

Aug. 4, 1931.

H. O. SIEGMUND

1,816,875

ELECTROLYTIC DEVICE

Filed April 27, 1927



INVENTOR  
HUMPHREYS O. SIEGMUND  
BY *J. G. Roberts*  
ATTORNEY

## UNITED STATES PATENT OFFICE

HUMPHREYS O. SIEGMUND, OF WEST ORANGE, NEW JERSEY, ASSIGNOR TO WESTERN ELECTRIC COMPANY, INCORPORATED, OF NEW YORK, N. Y., A CORPORATION OF NEW YORK

## ELECTROLYTIC DEVICE

Application filed April 27, 1927. Serial No. 187,068.

This invention relates to electrolytic devices, such as electrolytic condensers, and particularly to film forming electrodes therefor.

In manufacturing electrolytic condensers and other electrolytic devices, it has been the practice to employ aluminum of a very high degree of purity as a material for the film forming electrode or anode. This practice is followed chiefly for the reason that the presence of impurities in the aluminum tends to impair the film forming properties of the anode. For instance, the leakage resistance of the dielectric film of a condenser, the aluminum anode of which contains small amounts of other substances, such as those listed below, is considerably lower than that of a condenser the film forming electrode of which is of substantially pure aluminum. When the other substances contained in the film forming electrode are greater than 2% or 3%, the film forming properties of the electrode are so greatly impaired that its use is unsuitable even in apparatus designed for use with low voltages. When employing electrodes of substantially pure aluminum in electrolytic devices, the useful life of the device has been found in many cases to be very short due to the corrosion of the electrodes.

In accordance with the present invention there is provided for an electrolytic device a film forming electrode comprising mainly a film forming metal, such as aluminum, together with other materials, which may or may not be film forming, in such amounts that the ability of the electrode to resist corrosion is considerably increased. An electrode comprising between 98.0% and 99.4% aluminum and the rest other metals, such as those mentioned below, combined therewith, is characterized by a high resistance to corrosion as compared with the corrosion-resisting properties of an electrode formed of substantially pure aluminum and the film forming properties of such an electrode have been found to be satisfactory. If the film forming properties of the material are not thereby impaired, lower percentages of aluminum

may be employed. For instance, two or more film forming materials such as magnesium and aluminum may be combined in various proportions. In a preferred embodiment of the invention the following metals were combined with the pure aluminum in the amounts stated: Silicon 0.3%; manganese 0.05%; iron 0.30%.

The accompanying drawing shows an electrolytic condenser in which this invention has an embodiment. The condenser comprises a jar 1 for containing an electrolyte 2 in which an anode or film forming electrode 3 and a cathode 4 are positioned. While various electrolytes may be employed one which afforded satisfactory results was prepared from 450 grams boric acid, 75 c. c. ammonium hydroxide and 5 gallons distilled water. The cathode 4 is preferably non-film forming and may comprise aluminum together with sufficient other materials to render it substantially non-film forming as disclosed in Patent No. 1,578,857 of H. O. Siegmund et al, March 30, 1926. The anode 3 is composed chiefly of aluminum together with other materials in amounts which are insufficient to render the anode non-film forming. An anode comprising aluminum together with these materials is characterized by its increased ability to resist corrosion due to the action of the electrolyte, as compared with the corrosion-resisting properties of substantially pure aluminum. It has been found that a condenser employing an anode which comprises approximately 99.6% aluminum fails to function satisfactorily after a period of 3 or 4 months. While it has not as yet been determined just what the life of an electrolytic device will be when employing an anode composed of aluminum, with a low percentage of alloying materials, the results of tests made thus far indicate that it will be of the order of 6 or 7 years.

The following table shows the results of tests made on electrolytic condensers employing electrodes of aluminum with various amounts of other substances. These electrodes were immersed in an electrolyte of am-

monium borate for a period of more than 12 months and the percentage of failures noted:

| 5  | Per cent of — |         |           |      |        |        |                  |          |
|----|---------------|---------|-----------|------|--------|--------|------------------|----------|
|    | Failures      | Silicon | Manganese | Iron | Copper | Carbon | Total impurities | Aluminum |
| 10 | None          | 0.23    | 0.07      | 0.64 | 0.08   | 0.04   | 1.06             | 98.94    |
|    | 2.0           | 0.36    | 0.04      | 0.36 | Trace  | None   | 0.76             | 99.24    |
|    | 13.6          | 0.40    | 0.01      | 0.49 | Trace  | 0.03   | 0.93             | 99.07    |
|    | 30.0          | 0.13    | None      | 0.28 | None   | 0.04   | 0.45             | 99.55    |
|    | 39.0          | 0.05    | 0.03      | 0.50 | 0.08   | 0.04   | 0.70             | 99.30    |

While these tests do not afford sufficient data from which to determine with accuracy 15 the amount and kind of materials which can be contained in the the aluminum anode in order to obtain minimum corrosion together with satisfactory film forming properties, they do indicate that an anode comprising 20 between 98.0% and 99.4% aluminum will give satisfactory results. The alloying materials combined with the aluminum should preferably comprise one or more of the following: Silicon 0.2% to 1.5%; manganese 25 0.04% to 1.50%; iron 0.3% to 1.5%. Of these, it is believed that silicon is the most important.

The dielectric film formed on the anodes 30 of all of the condensers used in these tests was satisfactory initially. After the dielectric film was formed by applying a gradually increasing potential across the electrodes of the condenser, the leakage current at 40 volts 35 was found to be less than .035 amperes. The capacity of each of the condensers was about .001 farad and the resistance of each at 60 cycles was less than 1 ohm.

What is claimed is:

1. A film forming electrode for an electrolytic device comprising a film forming metal containing aluminum and having a small percentage of a substantially non-film forming metal combined therewith for improving the corrosion-resisting properties of 45 the electrode, said metal comprising silicon, manganese and iron.

2. A film forming electrode for an electrolytic device comprising between 98.0% and 99.4% pure aluminum, and small quantities of non-film forming materials including approximately .25% silicon.

3. A film forming electrode for an electrolytic device comprising an alloy, one of the constituents of which consists of between 55 98.0% and 99.4% pure aluminum, and another of which consists of approximately .25% silicon.

4. A film forming electrode for an electrolytic device comprising mainly pure aluminum and approximately .25% silicon.

5. A film forming electrode for an electrolytic device comprising mainly pure aluminum, small quantities of silicon and iron, 65 and between 0.04% and 1.5% manganese.

6. A film forming electrode for an electrolytic device comprising mainly pure aluminum, small quantities of silicon and manganese, and between 0.3% and 1.5% iron.

7. A film forming electrode for an electrolytic device comprising between 98.0% and 99.4% pure aluminum, a small quantity of manganese and approximately .25% silicon.

8. A film forming electrode for an electrolytic device comprising between 98.0% and 99.4% pure aluminum, small quantities of silicon and iron, and approximately .05% manganese.

9. A film forming electrode for an electrolytic device comprising mainly pure aluminum, together with a small amount of manganese, and approximately 0.3% iron and 0.8% silicon.

10. A film forming electrode for an electrolytic device comprising mainly pure aluminum, together with a small amount of iron, and approximately 0.3% silicon and 0.05% manganese.

11. A film forming electrode for an electrolytic device comprising mainly aluminum, together with approximately 0.3% silicon, 0.05% manganese and 0.3% iron.

In witness whereof, I hereunto subscribe my name this 27th day of April, A. D. 1927.

HUMPHREYS O. SIEGMUND.

100

105

110

115

120

125

130